

June 25, 1935.

C. H. KELLER

2,006,049

## CONCENTRATION OF ORES BY FLOTATION

Filed July 27, 1932

Fig. 1.



Fig. 2. } 4



## UNITED STATES PATENT OFFICE

2,006,049

## CONCENTRATION OF ORES BY FLOTATION

Cornelius H. Keller, San Francisco, Calif., assignor to Minerals Separation North American Corporation, New York, N. Y., a corporation of Maryland

Application July 27, 1932, Serial No. 624,965

7 Claims. (Cl. 209—166)

This invention relates to the concentration of ores by flotation, and is herein illustrated as applied to a variety of ores.

According to the form of the present invention disclosed in detail, pulps of the ores are treated with small amounts of free sulphur-containing acids, such as xanthic acids, and the usual flotation agents, with the result that recovery is enhanced, or a richer concentrate is obtained, or 10 both of these results are achieved.

To achieve these results it is important to follow the correct methods of introducing the free xanthic or other acids.

According to one method the free xanthic acid 15 was made by dissolving a sodium or potassium xanthate in water and adding its equivalent amount of a stronger acid, usually sulphuric, in diluted form, immediately before addition to the agitated pulp.

According to a second method the fresh xanthic acid was introduced by producing it in an enclosed vessel below the pulp level in the flotation machine and discharging the xanthic acid immediately into the surrounding pulp. This procedure was deemed of especial value because the conspicuous odor of these unstable xanthic acids indicated a sensible loss if ordinary methods of introduction were employed. For this, and other reasons, extraordinary precautions had to be employed to obtain the best results.

According to a third method, the free acid was made by dissolving or suspending a sodium or potassium xanthate in the corresponding alcohol, and an equivalent proportion of acid, usually sulphuric acid, was introduced, and the resulting alcoholic material added immediately to the agitated pulp, either in the flotation machine or at the grinding mill, as required.

It has been found that good results may be obtained in acid as well as in alkaline circuits by such methods of introducing sulphur-containing acids to the pulp.

In some instances xanthic acids carrying more than three carbon atoms in their molecule, have 45 proved especially useful, as, for example, the xanthic acids made from the higher aliphatic alcohols, such as butyl or amyl, or the cyclic alcohols, such as benzyl or cyclohexanyl.

In the accompanying drawing, Figure 1 is a 50 section through a flotation machine showing one method of introducing the reagent.

Figure 2 is a diagram showing how various proportions of one of the reagents varies the results in concentrating one typical ore.

55 Nevada Consolidated Copper ore was wet ground

with five pounds of calcium oxide per ton, diluted with added water and agitated with 0.1 pound of pine oil, and 0.0075 pound of potassium ethyl xanthate converted to ethyl xanthic acid, all per ton of ore. The xanthic acid was produced by reacting on an aqueous solution of the potassium xanthate with an equivalent proportion of sulphuric acid, producing about three-fourths as much xanthic acid as xanthate, and adding the xanthic acid immediately to the agitated ore pulp 10 below the surface. The pulp was then agitated two minutes and a froth concentrate separated for five minutes.

The concentrate was 4.95% of the weight of the heads. The heads contained 1.33% of copper, 15 the concentrate contained 25.32% copper, and the tailings 0.08% copper, representing a recovery of 94.3%. The recovery and grade were both greater than were obtained when potassium ethyl xanthate was used, as such.

20 The fresh xanthic acid was advantageously introduced into the ore pulp by immersing in the pulp in the spitzkasten 1 of the flotation machine 2 a glass bottle 3 carrying an aqueous solution of the potassium salt of the desired xanthic acid. 25 The desired acid was produced by pouring the theoretical equivalent of sulphuric acid into a thistle tube 4 passing through the rubber stopper 5 to almost the bottom of the bottle 3. The acid was immediately followed by wash water in sufficient quantity to wash the acid out into the pulp through a bent tube 6 just passing through the cork 5 and bent horizontally so as to flow the xanthic acid horizontally into the pulp which was in the meantime agitated by the usual propeller 7 at 30 the bottom of the agitation box 8.

A series of parallel tests on the same ore with varying amounts of ethyl xanthic acid used under parallel conditions yielded the results tabulated below:

| Xanthic acid          | Concentrate          | Assays  |                  |         | Recovery |
|-----------------------|----------------------|---------|------------------|---------|----------|
|                       |                      | Heads   | Concen-<br>trate | Tails   |          |
| Added lbs.<br>per ton | Percent by<br>weight | Percent | Percent          | Percent | Percent  |
| 0.038                 | 8.14                 | 1.29    | 15.04            | 0.07    | 95.1     |
| 0.015                 | 7.1                  | 1.33    | 17.76            | 0.07    | 95.1     |
| 0.0075                | 5.3                  | 1.32    | 23.60            | 0.07    | 95       |
| 0.0038                | 4.6                  | 1.35    | 27.44            | 0.09    | 93.6     |
| 0.0015                | 4.6                  | 1.35    | 24.80            | 0.22    | 84.5     |

These results, plotting richness of concentrate and recovery against the amount of xanthic acid used, as shown in the curves of Fig. 2, indicate 55

that the maximum richness of concentrate for this ore was attained at about 0.0038 pounds of xanthic acid per ton, with the aid of other flotation agents.

- 5 When amyl, and secondary butyl xanthic acids were substituted for ethyl xanthic acid in the treatment of Nevada Consolidated ore, other conditions remaining the same, equally good results were obtained; in fact the concentrates were 10 slightly richer when using the amount of xanthic acid formed by acidifying 0.0075 pounds per ton of the corresponding potassium xanthates.

It was found that slightly better recoveries or richer concentrates were obtained with ethyl and 15 amyl xanthic acids when the acid was made by acidifying the corresponding xanthate with sulphuric rather than acetic acid, although a butyl xanthic acid prepared with acetic acid was more efficient than one prepared with sulphuric acid.

- 20 Fresh furfuryl xanthic acid prepared by adding acetic acid to an aqueous solution of potassium furfuryl xanthate was used in concentrating Nevada Consolidated as follows:

The ore was reground for 7 minutes from 10-25 mesh with 5 pounds of calcium oxide per ton, made into a pulp with added water and agitated with 0.1 pound of pine oil and a calculated 0.05 pound of the fresh furfuryl xanthic acid. The pulp was then agitated two minutes and a froth 30 concentrate separated for five minutes.

The concentrate was 5.63% of the weight of the heads. The heads contained 1.36% copper, the concentrate 22.56%, and the tailing 0.1% of copper, representing a recovery of 93.1%.

- 35 Fresh furfuryl xanthic acid prepared by adding sulphuric acid to an aqueous solution of potassium furfuryl xanthate, in a parallel test, yielded the following results:

The concentrates were 5.12% the weight of the 40 heads. The heads contained 1.36% copper, the concentrate 24.64% and the tailings 0.11% of copper, representing a recovery of 92.4%.

Nevada Consolidated Copper ore was ground with five pounds of calcium oxide, per ton, made 45 into a pulp with added water and agitated with 0.1 pound of pine oil and with freshly made benzyl xanthic acid, made by acidifying with dilute sulphuric acid 0.005 pound of potassium benzyl xanthate, all per ton of ore. The pulp was agitated for two minutes and then a froth concentrate separated for six minutes. The concentrate was 4.71% of the weight of the heads. The heads contained 1.376% copper, the concentrate 23.76%, and the tailings 0.27% copper, representing 55 a recovery of 81.3%.

When 0.01 pound of the potassium benzyl xanthate were substituted for the 0.005 pound in a parallel test with heads containing 1.364% copper, a concentrate was obtained equal to 4.91% 60 of the heads. The concentrate contained 25.44% copper, and the tailings 0.12% copper representing a recovery of 91.6%.

Nevada Consolidated Copper ore was ground with five pounds of calcium oxide, per ton, made 65 into a pulp with added water and agitated with 0.1 pound of pine oil and with freshly made cyclohexanol xanthic acid made by acidifying with dilute sulphuric acid 0.005 pound of potassium cyclohexanol xanthate, all per ton of ore. The pulp was agitated for two minutes and then a froth concentrate separated for six minutes. The concentrate was 4.73% of the weight of the heads. The heads contained 1.359% copper, the 70 concentrate 24.32% and the tailings 0.22% copper, representing a recovery of 84.6%

When 0.01 pound of the potassium cyclohexanol xanthate was substituted for the 0.005 pound in a parallel test with heads containing 1.363% copper, a concentrate was obtained equal to 4.23% of the heads. The concentrate contained 26.64% copper, and the tailings 0.11% copper, representing a recovery of 92.3%.

When Clay Mine ore of Phelps Dodge Corporation was wet ground with 5 pounds calcium oxide, diluted with water and agitated with 0.15 pound of pine oil and 0.05 pound of cresylic acid, and with fresh xanthic acid made by adding sulphuric acid to 0.02 pound of potassium ethyl xanthate, all per ton of ore, the following results were obtained by agitating two minutes and separating 15 froth for ten minutes.

The concentrates were 11.1% of the weight of the heads. The heads contained 0.87% of copper, the concentrate 6.96% copper, the tails 0.11% copper, representing a recovery of 88.8%. 20 This may be compared with a concentrate containing 6.48% copper and a tailing of 0.13% copper when the corresponding amount of potassium xanthate was substituted for the xanthic acid.

When Miami Copper Company ore was wet ground with 3 pounds of calcium oxide, diluted with added water, and agitated with 0.1 pound of pine oil and with fresh xanthic acid made by adding sulphuric acid to 0.0075 pound of potassium ethyl xanthate, all per ton of ore, the following results were obtained by agitating two minutes and separating froth for five minutes.

The concentrates were 4.1% of the weight of the heads. The heads contained 0.72% copper, 35 the concentrate 14%, and the tailings 0.15% copper, representing a recovery of 80%. The richest concentrate obtained when potassium xanthate was used was just over 11% copper.

When less xanthic acid was used, equivalent to 40 0.005 pound per ton of potassium ethyl xanthate, a concentrate was obtained containing 14.96% of copper, with a recovery of 78.7%.

Ethyl xanthic acid, amyl xanthic acid, butyl xanthic acid, all proved useful in connection 45 with Morenci ore of Phelps-Dodge Corporation.

When the Morenci ore was wet ground with 5 pounds calcium oxide, with added water and agitated with 0.1 pound of pine oil and with fresh ethyl xanthic acid made by adding sulphuric acid 50 to 0.05 pound of potassium ethyl xanthate, all per ton of ore, the following results were obtained:

The concentrates were 10.7% of the weight of the heads. The heads contained 1.69% copper, the concentrate 14.08%, and the tailings 0.20% 55 copper, representing a recovery of 89.4%.

A richer concentrate with a lower recovery was obtained when 0.01 pound of potassium ethyl xanthate was used for producing the xanthic acid instead of the 0.05 pound just described.

When another lot of the same Morenci ore was similarly concentrated, using 0.025 pound of potassium amyl xanthate, so as to yield amyl xanthic acid, the results were as follows:

The concentrates were 9.8% of the weight of 65 the heads. The heads contained 1.74% copper, the concentrate 15.88%, and the tailings 0.20% copper, representing a recovery of 89.6%.

A richer concentrate containing 16.32% of copper, with a recovery of 84.4%, was obtained when 70 the smaller amount 0.01 pound of potassium amyl xanthate was used to produce the amyl xanthic acid.

When another lot of the same Morenci ore was similarly concentrated, using 0.025 pound po- 75

tassium butyl xanthate, so as to yield butyl xanthic acid, the results were as follows:

The concentrates were 11% of the weight of the heads. The heads contained 1.77% copper, 5 the concentrate 14.32% and the tailings 0.22% copper, representing a recovery of 84.8%.

When another lot of the same Morenci ore was similarly concentrated, substituting 0.05 pound 10 of potassium furfuryl xanthate for the ethyl xanthate, the results were as follows:

The concentrates were 9.3% of the weight of the heads. The heads contained 1.74% of copper, the concentrate 16.16%, and the tailings 0.26%, representing a recovery of 86.4%.

15 Parallel improvement in concentration was obtained when other acids than xanthic acids were introduced into ore pulps.

Nevada Consolidated Copper ore was ground with five pounds of calcium oxide, per ton, made 20 into a pulp with added water and agitated with 0.1 pound of pine oil and with freshly made dibutylthiophosphoric acid, made by acidifying with dilute sulphuric acid 0.02 pound of the commercial compound known as #208 aerofloat, all 25 per ton of ore. The pulp was agitated for two minutes and then a froth concentrate separated for five minutes.

The concentrate was 4.62% of the weight of the heads. The heads contained 1.41% copper, 30 the concentrate 27.20%, and the tailings 0.16% copper, representing a recovery of 89.2%.

The 27.2% copper in the concentrate compared favorably with the best, 25.28% of copper obtained by parallel test procedures in which the 35 sodium salt, #208 aerofloat, was used instead of the acid, and the recovery was greater, with the same proportion of copper in the tailing in both tests.

When another lot of the same Nevada Consolidated ore was similarly concentrated, substituting 40 0.006 pound of the #208 aerofloat for the 0.02 pound, to make dibutylthiophosphoric acid, the results were as follows:

The concentrate was 4.84% of the weight of 45 the heads. The heads contained 1.34% of copper, the concentrate 25.04%, and the tailings 0.13% copper, representing a recovery of 90.7%.

An even better grade of concentrate, 25.84%, was obtained when concentration was effected 50 with the aid of 0.004% of the #208 aerofloat converted to the acid, though the recovery was less, viz., 86.2%.

When the same ore was concentrated by the aid of diethylthiophosphoric acid made by treating 55 commercial sodium aerofloat with dilute sulphuric acid, the concentrate was usually richer or the tailings carried less copper than when the ore was concentrated with a corresponding amount of the unchanged sodium aerofloat.

60 When a fresh sample of Utah Copper Company ore was concentrated by grinding with 6 pounds of calcium oxide and 0.25 pound sodium cyanide, both per ton, diluted with added water, and agitated with 0.4 pound cresylic acid and diethyl-65 dithiophosphoric acid made by treating 0.04 pound sodium aerofloat with dilute sulphuric acid, both per ton, the following result was obtained:

The concentrate was 5.55% of the weight of 70 the heads. The heads contained 0.97% copper, the concentrate 13.44% and the tailings 0.24% copper, representing a recovery of 77.8%. This compared with a parallel test of the same ore, substituting the sodium aerofloat for the diethylthiophosphoric acid, in which heads carrying 75 0.95% copper yielded a concentrate car-

rying 11.68% copper and a tailing of 0.23% copper,—a slightly poorer recovery and an inferior concentrate.

When the xanthic acid was made by dissolving or suspending a xanthate in the corresponding alcohol and treating with an equimolecular proportion of acid, an agent was obtained which often proved extraordinarily useful for assisting in the production of rich concentrates or large recoveries in ore concentration. Some of 10 the results are shown in the following examples:

In a series of tests Nevada Consolidated copper ore was reground for 7 minutes from 10-mesh with 5 pounds of calcium oxide per ton in a laboratory ball mill, diluted with added water 15 and agitated with 0.05 pound xanthic acid carried in ethyl alcohol and 0.1 pound pine oil, both per ton of ore. After 2 minutes agitation a froth concentrate was separated for 5 minutes.

In one test the calculated amount of xanthic acid was prepared by adding acetic acid to amyl alcohol carrying 10% potassium amyl xanthate. The concentrate was 5.4% of the weight of the heads. The heads contained 1.35% copper, the concentrate 23.84%, and the tailings 0.07% copper, representing a recovery of 95.1%.

In another test the calculated amount of xanthic acid was prepared by adding hydrochloric acid to amyl alcohol carrying 10% potassium amyl xanthate. The concentrate was 5.43% of the weight of the heads. The heads contained 1.34% of copper, the concentrate 23.44%, and the tailings 0.07% copper, representing a recovery of 95.1%.

In another test the calculated amount of xanthic acid was prepared by adding sulphuric acid (in half equimolecular proportion) to butyl alcohol carrying 10% potassium butyl xanthate. The concentrate was 5.52% of the weight of the heads. The heads contained 1.34% copper, the concentrate 23.28% and the tailings 0.06% copper, representing a recovery of 95.7%.

Almost as good results as the foregoing were obtained when the xanthic acid used was ethyl xanthic acid obtained by adding acetic acid to 45 potassium ethyl xanthate carried in ethyl alcohol, and when the acid used was the acid obtained by adding sulphuric acid to potassium furfuryl xanthate carried in furfuryl alcohol.

Xanthic acids also proved useful with ores carrying other metals. The furfuryl xanthic material was found to increase both the grade of concentrate and the recovery of zinc in the concentration of a zinc ore.

A pulp of Joplin zinc ore was agitated with 1.5 pounds copper sulphate, Barrett #634 0.2 pound, pine oil 0.3 pound, and the acid by adding the theoretical equivalent of sulphuric acid to 0.2 pound potassium furfuryl xanthate, all per ton 55 of ore. After agitating for two minutes a froth concentrate was separated for five minutes.

The results were as follows: The concentrates were 21.1% of the weight of the heads. The heads contained 14.29% of zinc, the concentrates 62.0%, and the tailings 1.5%, representing a recovery of 91.7%. The best results with the corresponding xanthate were a concentrate containing 60.8% zinc with a 1.9% tailing.

A partially oxidized copper ore from the Chile Exploration Company, Antofagasta, Chile, was ground wet in a ball mill, diluted with more water and agitated in a flotation machine. To this pulp were added 0.15 lb. of cresol per ton of ore, 70 and the xanthic acid corresponding to 0.2 pound 75

of potassium ethyl xanthate per ton, made by acidifying the xanthate in solution with its equivalent of dilute sulphuric acid and immediately adding the mixture to the agitated pulp.

- 5 Froth was removed for 5 minutes, yielding the first concentrate. The pulp was then agitated for 5 minutes with the further addition of 0.15 pound of cresol, 0.25 pound of Barrett No. 4, and 2.0 pounds of potassium xanthate separately converted to xanthic acid as above, all per ton of ore, and a second froth concentrate removed.

10 The result is shown in the following tabulation:

| 15 | Product              | Weight | Copper  |         | Recovery |          | Percent | Ounces | Percent |
|----|----------------------|--------|---------|---------|----------|----------|---------|--------|---------|
|    |                      |        | Total   | Oxide   | Total Cu | Oxide Cu |         |        |         |
|    |                      |        | Percent | Percent | Percent  | Percent  |         |        |         |
| 20 | Heads.....           | 100.00 | 2.35    | 0.64    | 100.0    | 100.0    | 100.0   | 0.289  | 100.0   |
|    | 1st concentrate..... | 8.70   | 15.20   | 1.92    | 56.1     | 26.2     | 3.2     | 8.35   | 92.4    |
|    | 2nd concentrate..... | 6.77   | 13.52   | 5.98    | 38.9     | 63.2     | 6.1     | 0.14   | 2.9     |
|    | Tailings.....        | 84.53  | 0.14    | 0.08    | 5.0      | 10.6     | 90.7    | 0.015  | 4.7     |

15 Amyl xanthic acid was used in concentrating a lead ore as follows:

- 25 A pulp of Deslodge Lead Company ore was agitated with 0.1 pound pine oil and amyl xanthic acid made by adding the theoretical equivalent of dilute sulphuric acid to an aqueous solution carrying 0.05 pound per ton of potassium amyl xanthate, and a froth concentrate separated. The xanthic solution was mixed with the acid immediately before adding to the agitated pulp.

30 The results were as follows:

- 35 The concentrates were 8.93% of the weight of the heads, the heads contained 4.65% of lead, the concentrates 50% and the tailings 0.2% of lead, representing a recovery of 96.1%.

Morning Mine lead-zinc ore was concentrated by wet grinding for 20 minutes with 0.2 pound 40 sodium cyanide and 1 pound zinc sulphate, both per ton of ore, diluting with added water, and agitating the pulp with 0.2 pound cresyllic acid to yield a lead float. The remaining pulp was agitated with 1 pound copper sulphate, 0.2 pound 45 Barrett #4, and 0.05 pound pine oil, all per ton of ore, to yield a zinc float. In addition to the foregoing there was added, at the beginning of the agitation, amyl xanthic acid made by adding the theoretical equivalent of sulphuric acid to 50 0.025 pound potassium amyl xanthate, per ton of the ore.

55 The weight of the lead concentrate was 17% of the heads and of the zinc concentrate 9.0% of the heads. The heads contained 9.26% lead and 5.9% zinc. The lead concentrate contained 52.6% lead, and the zinc concentrate 40.2% zinc. The tailings contained 0.1% of lead and 0.3% of zinc, representing a recovery of 96.7% of lead and 61.5% zinc in their respective concentrates.

60 A pulp of Mexican Candelaria silver ore was agitated with 0.1 pound pine oil and amyl xanthic acid made by adding the theoretical equivalent of sulphuric acid to 0.1 pound potassium xanthate, both per ton of ore, and a froth concentrate separated.

65 The heads contained 35.73 ounces of silver per ton, the concentrates 1068.9 ounces, and the tailings 4.9 ounces, representing a recovery of 86.7%.

70 Gold ore from the Central Eureka Mining Company of Sutter Creek, California, was reground wet from 10 mesh until 0.4% was +65 mesh and 71.2% was -200 mesh, diluted with added water and agitated with 0.5 pound Barrett No. 4, 0.15

10 pound Yarmor pine oil, and fresh amyl xanthic acid made by acidifying with sulphuric acid 0.4 pound potassium amyl xanthate, all per ton of ore, and a rougher froth concentrate separated. The rougher concentrate thus obtained was retreated to yield a finished concentrate and a middling. The results are shown in the following table:

|                   | Weight  | Au     | Recoveries | 10      |
|-------------------|---------|--------|------------|---------|
|                   | Percent | Ounces | Percent    | Percent |
| Heads.....        | 100.0   | 0.289  | 100.0      |         |
| Concentrates..... | 3.2     | 8.35   | 92.4       |         |
| Middlings.....    | 6.1     | 0.14   | 2.9        |         |
| Tailings.....     | 90.7    | 0.015  | 4.7        | 15      |

15 When the potassium amyl xanthate was replaced by potassium butyl xanthate to yield the corresponding xanthic acid in a parallel test, the following results were obtained:

|                   | Weight  | Au     | Recoveries | 20      |
|-------------------|---------|--------|------------|---------|
|                   | Percent | Ounces | Percent    | Percent |
| Heads.....        | 100.0   | 0.287  | 100.0      |         |
| Concentrates..... | 3.4     | 7.78   | 92.2       |         |
| Middlings.....    | 5.6     | 0.24   | 4.6        |         |
| Tailings.....     | 91.0    | 0.01   | 3.2        | 25      |

30 Having thus described certain embodiments of the invention, what is claimed is:

1. The process of concentrating an ore which consists in dispersing in an alkaline ore pulp, an appreciable amount of separately prepared free xanthic acid but in a proportion of less than 0.05 pound per ton of solids in the pulp, agitating such pulp with a further agent such as will produce a floating concentrate, and separating the float.

2. The process of concentrating an ore which consists in dispersing in an alkaline ore pulp free xanthic acid carrying more than three atoms of carbon in the molecule, agitating such pulp with a further agent such as will produce a floating concentrate, and separating the float.

3. The process of concentrating an ore which consists in dispersing in an alkaline ore pulp free xanthic acid made from an aliphatic alcohol and carrying more than three atoms of carbon in the molecule, agitating such pulp with a further agent such as will produce a floating concentrate, and separating the float.

4. The process of concentrating an ore which consists in dispersing in an ore pulp free xanthic acid made from a cyclic alcohol, agitating such pulp with a further agent such as will produce a floating concentrate, and separating the float.

5. The process of concentrating an ore which consists in dispersing in an ore pulp free furfuryl xanthic acid, agitating such pulp with a further agent such as will produce a floating concentrate, and separating the float.

6. The process of concentrating an ore which consists in dispersing in an alkaline ore pulp free furfuryl xanthic acid, agitating such pulp with a further agent such as will produce a floating concentrate, and separating the float.

7. The process of concentrating an ore which consists in dispersing in an ore pulp alcohol carrying a freshly prepared free xanthic acid, agitating with such other agent as will produce a floating concentrate, and separating the float.